

# United States Patent Office

2,698,230

Patented Dec. 28, 1954

1

2,698,230

## MAGNESIUM BASE ALLOYS CONTAINING ZIRCONIUM

William Michael Doyle, Slough, England, assignor, by mesme assignments, to Magnesium Elektron Limited, near Manchester, England, a company of England

No Drawing. Application February 12, 1951,  
Serial No. 210,627

Claims priority, application Great Britain  
February 21, 1950

2 Claims. (Cl. 75—168)

This invention relates to magnesium base alloys containing zirconium and has for one of its purposes to provide a method of making such alloys.

It is another object of this invention to provide means for facilitating or rendering possible the introduction of zirconium into magnesium base alloys in a particularly effective manner.

It is a special object of this invention to provide an agent, being a fused mixture of a zirconium compound and an alkali compound, adapted to alloy zirconium with magnesium metal or with a magnesium-base alloy.

It is also an object of this invention to provide a new method of preparing such agent.

I am aware that it has been proposed to introduce zirconium into magnesium base alloys by adding to the molten magnesium under stirring such alloying salts as zirconium tetrachloride, or fused mixtures of zirconium tetrachloride and potassium and sodium chlorides. A disadvantage in either case is that serious losses of zirconium tetrachloride occur due to volatilisation. Another disadvantage of this way of proceeding is that fairly large amounts of magnesium chloride are formed, which, together with the alloying zirconium salts, being very fluid at the alloying temperatures, envelop the fine particles of the elemental zirconium forming by reduction so that the zirconium metal is not "available" to carry out the function of grain refining and alloying. Furthermore, separation of the alloying salt from the molten metal is very poor so that a very large percentage of the alloy has to be discarded. In general, castings made by these techniques possess inconsistent tensile properties, and they are prone to be commercially unsatisfactory due to finely disseminated magnesium chloride or alloying salt inclusions, which impair the corrosion resistance of the magnesium-zirconium alloy.

Other methods have been suggested involving the use of zirconium tetrafluoride, or double salts of zirconium tetrafluoride and a potassium halide, but the zirconium tetrafluoride is more expensive and is less readily obtainable than zirconium tetrachloride. Also, the commercial grade of zirconium tetrafluoride is usually the monohydrate of this salt, or a complex addition compound containing the  $H_2O$  radicle. It is very difficult to remove this hydroxyl radicle from the salt without oxidising the zirconium and, in any case, the procedure involved is very expensive.

As a result of considerable research, I have developed a technique whereby a compound or complex salt containing zirconium tetrachloride can be used to introduce the zirconium into the alloy while avoiding the aforementioned disadvantages.

I have found that an exothermic reaction occurs between zirconium tetrachloride and potassium fluoride, and that use can be made of this phenomenon provided precautions are taken to contain the momentary sublimation of the zirconium salt, which occurs just prior to the mixture becoming completely molten. I have also found that the addition of zirconium tetrachloride to potassium fluoride progressively lowers the melting point and that, when the weight ratio of  $ZrCl_4:KF$  lies between approximately 0.75:1 and 4:1, the melting points of the resulting mixtures lie between 500° and 400° C., approximately. I have further found that compound salts of such mixtures can be raised to a temperature of 650° C., without noticeable loss of zirconium tetrachloride by volatilisation. In fact, volatilisation of the zirconium salt at this temperature is only noticeable when the ratio of  $ZrCl_4:KF$  is about 5:1 or greater.

Accordingly, my invention provides a compound salt comprising essentially a fused mixture of zirconium tetrachloride and potassium fluoride within the weight ratio of 0.75:1 and 4:1.

My invention further provides methods of making such a salt mixture and of making with the use of such a salt mixture magnesium base alloys containing zirconium.

I prefer to make the salt mixture or compound salt in the following manner: The potassium fluoride is first dried and a proportion of this salt and of the zirconium tetrachloride are intimately mixed in the bottom of a warm (less than 150° C.) crucible in the ratio of approximately, two parts by weight of zirconium tetrachloride to one part by weight of potassium fluoride. This intimate mixture is used to "trigger" or initiate the reaction and the amount of the salts used for this purpose may be up to 25% of the whole. Then the remainder of part of the desired amounts of these salts are mixed or placed in the crucible in alternate thin layers, leaving for the final addition sufficient potassium fluoride to form a thin layer on the top. The potassium fluoride layer on the top of the mixture will automatically form a high-melting crust which will prevent excessive loss of zirconium tetrachloride during the reaction. The crucible should be fitted with a close-fitting, fairly heavy lid having a vent hole formed therein. Gentle heat is applied to the bottom of the crucible and, when the exothermic reaction occurs, the bulk of the salts decreases to about a quarter of the original volume, and forms a pool of molten mixed salts. The crust formed by the potassium fluoride on the top may then be broken and stirred in.

In making up the compound salt, according to the technique described above, and when the ratio in the final mixture of zirconium tetrachloride to potassium fluoride is to be near 4 to 1, it is desirable to ensure that in the body of the charge this ratio is not exceeded, which normally would be the case after deducting the "trigger" portion as aforesaid. To avoid such excess, some of the zirconium tetrachloride may be withheld until the main mixture is molten. Similarly, when the ratio of zirconium tetrachloride to potassium fluoride is to be near the lower limit of 0.75 to 1, it is desirable to withhold some of the potassium fluoride from the main charge until this charge is molten, in order to ensure that the ratio in the body of the charge is near say 1.5 to 1. A mixture of two parts by weight of zirconium tetrachloride and one part by weight of potassium fluoride made up as described above will be molten at about 420° C.

For the purposes of description I shall refer to the fused mixture of only zirconium tetrachloride and potassium fluoride as the "compound" salt, such a salt containing from about 43 to 80% zirconium tetrachloride, the remainder being potassium fluoride, substantially as hereinafter described for the introduction of zirconium into magnesium and magnesium alloys which do not contain inhibiting elements that form high-melting compounds with zirconium. However, I refer to modify this mixture, in order to make it more suitable for the alloying of zirconium to magnesium alloys in the foundry, by making certain additions of other salts or compounds to improve its physical characteristics, and the resulting fused mixture will be called the "complex" salt.

The amount of zirconium tetrachloride contained in the fused complex salt must be adequate to ensure that this salt contains sufficient zirconium to function as a practical and economic source of this metal in the subsequent alloying operation in the foundry. I prefer the amount of zirconium tetrachloride to be between 24 and 60% by weight of the complex salt. With this object in view, when making up the complex salt, I prefer to maintain the weight ratio of  $ZrCl_4:KF$  in the compound salt portion of the said complex salt within the limits of 1.5:1 and 2.5:1. Between these limits, the choice of the ratio to be used, and therefore the amount of zirconium tetrachloride in the complex salt, will be controlled by the

total amount of the other constituents as described hereinafter.

In order to ensure that the specific gravity of the final complex salt, when molten, may be sufficiently high that it will remain at the bottom of the crucible during the alloying process, and give good separation between it and the molten metal, I prefer to add to the compound salt a heavy salt, such as dry anhydrous barium chloride. The preferred amount of barium chloride is from 0 to 30% by weight of the whole. About 10% of barium chloride results in the fused complex salt having a specific gravity in excess of 2.0. Up to two-thirds of the required amount of barium chloride may be replaced by barium fluoride.

The complex salt may contain up to 20% of magnesium fluoride as an inspissating agent or thickener, in order to decrease its fluidity at the alloying temperature of about 800° C. When magnesium fluoride is used for this purpose, I prefer to calcine it at a temperature between 600-800° C. for up to 3 hours in order to drive off moisture and other volatile constituents (which may be present in commercial magnesium fluoride up to a figure as high as 20 per cent). If this calcining operation is not carried out, the addition of magnesium fluoride gives rise to frothing and bubbling of the molten salt, and the zirconium becomes oxidised and therefore "unavailable" for alloying purposes. The grade of commercial magnesium fluoride which is stated to contain up to 15% or more of calcium fluoride, may be used. Other inspissating agents which may be present, are aluminium fluoride up to 6%, and calcium fluoride up to 10%. The presence of magnesium oxide, even when used in the calcined condition, is harmful, as it oxidises the zirconium and reduces the "available" zirconium content of the salt. As an impurity, it would not be economical to tolerate more than 1% of magnesium oxide.

The most useful inspissating compound which I have found, is zirconium oxide, because it offers three advantages. Firstly, when used in amounts up to about 25%, it has a definite, but controllable inspissating effect which is a function of the amount used. I prefer to add between 10 and 25 per cent of the oxide. Additions greater than 25 per cent tend to make the complex salt too thick and viscous, so that it is unworkable at the alloying temperature. Secondly, it is very dense and it increases the specific gravity of the complex salt, so that all or part of the barium chloride or barium chloride-barium fluoride addition may be replaced. Thirdly, when added during the make-up of the complex salt according to the technique which will be described hereafter, it controls the reactivity of the zirconium tetrachloride during the exothermic reaction with the potassium fluoride.

Within the limits stated above, the various inspissating agents may be used together, but their total should not exceed 30 percent by weight of the complex salt. Also, in order to avoid oxidation of the zirconium, they should be dried, before use, at a temperature of at least 110° C.

Other reducible halide salts of desirable alloying additions may also be added to the complex salt. For example, the presence of small amounts of beryllium in magnesium alloys considerably reduces the tendency to oxidation and burning of the molten metal at the high temperatures required for the zirconium alloying operation. Therefore, beryllium chloride or fluoride or the potassium double salts of these compounds may be added to the complex salt to the extent of up to about 7% by weight. The amount of the beryllium salt to be added must be carefully controlled, because beryllium in magnesium tends to enlarge the grains and therefore, to this extent, counteracts the beneficial effects of zirconium.

I have found that the reactivity of zirconium tetrachloride varies with the source of the supply and, when making up large melts of the complex salt, some of this material may react violently with the potassium fluoride, giving rise to a loss of zirconium salt by sublimation. However, if the potassium fluoride, except that portion of this salt which is used with zirconium tetrachloride to "trigger" the reaction, is mixed with all or part of the required addition of zirconium oxide, then the complex salt may be made up as hereinbefore described for the compound salt and the zirconium oxide will then control or dampen the reaction which then proceeds quietly. The "trigger" portion is the mixture of zirconium tetrachloride and potassium fluoride in the ratio of 2:1 by weight, which is placed in the bottom of the crucible to initiate

the reaction. It is calculated on the basis of using for this purpose between 5 per cent and 25 per cent of the required zirconium tetrachloride content of the complex salt and 10 per cent is sufficient as a rule.

When the so-called crude or unrefined grade of zirconium tetrachloride powder is used for making up the alloying salt, due allowance must be made for the zirconium oxide content and the zirconium oxide portion of the oxychloride content of this material, when deciding on the addition of zirconium oxide to be made, either for inspissation or for dampening the exothermic reaction.

When the exothermic reaction is complete and the required amounts of zirconium tetrachloride, potassium fluoride and zirconium oxide are in the form of a molten pool in a crucible or other suitable container, the desired amounts of the other ingredients, for example, additional inspissating agents and barium chloride or fluoride salts, are added and thoroughly mixed into the mass.

In making up the complex salt, it is desirable to maintain the temperature as low as possible in order to keep the oxidation of the zirconium salt to a minimum.

When molten and thoroughly mixed, the hereinbefore described compound or complex salt may be poured directly into the molten magnesium or magnesium alloy, to which it is intended to add zirconium, and the metal temperature may be raised to between 760-820° C., the salt being stirred in for about 1-10 minutes, after which the metal is allowed to settle, while maintaining the temperature within this range. This settling period, which may be up to 20 minutes, or even longer, provided the temperature is maintained, is necessary so that all the impurities and traces of high melting point compounds of zirconium and flux inclusions may settle to the bottom. It is essential that burning or oxidation of the metal should be prevented as far as possible during the melting and alloying procedure by the use of a high-melting point, magnesium chloride-free, heavy flux, similar to that used for the melting of cerium-containing magnesium alloys in bale-out or "sulphur-dome" furnaces. This flux is carefully removed from the top of the metal and from the sides of the crucible immediately before the commencement of the final settling operation and, from then on, oxidation of the molten metal is prevented by dusting with sulphur or suitable compound composed of a mixture of sulphur and boric acid.

I, however, prefer to cast all the fused compound or complex salt into thick slab moulds, whereupon it is broken up into suitably sized pieces. These pieces or lumps of fused salt are then placed in the bottom of the crucible, in which it is intended to carry out the alloying, and the magnesium ingots are placed on top, or molten magnesium is poured over the salt. After alloying in the normal way with the desired alloying metals, other than zirconium, the temperature of the magnesium or magnesium alloy is raised to 760-820° C. as before, and the salt is stirred in by hand with a suitable stirrer, or a mechanical device may be used. The same type of flux as described above should be used to protect the metal from burning, and after stirring for 1-10 minutes and removal of the flux, the metal should be allowed to settle as before.

The desired other alloying metals referred to above may be the non-inhibiting elements zinc, cadmium, silver, thallium, thorium, copper, bismuth, beryllium, lead, lithium, calcium, cerium or other rare-earth metal or cerium-mischmetall or other combinations of the rare-earth metals.

I have found that it is advantageous to repeat the stirring and settling operations, especially when the salt is being used for the first alloying with magnesium. A definite increase in the zirconium content of the metal occurs during the second stirring after the initial stirring and settling operation. This procedure may be repeated a third or fourth time if necessary. When a multiple stirring and settling technique is used, the flux may be left on the top of the metal to protect it from burning until immediately prior to the final settling operation, when it is carefully removed from the surface of the melt and from the sides of the crucible as before.

The compound or complex salt may also be used for revivifying magnesium alloys containing zirconium which require to be remelted, before being cast into suitable castings or shapes. The amount of salt required for initial alloying or revivifying purposes is a function of

the available zirconium content of the salt and that required in the finished alloy, but I have found that it is preferable to arrange the available zirconium content of the salt so that an amount of salt equivalent to about 5-25% by weight of the metal would be required.

In order to produce the optimum reduction in the grain-size and the corresponding improvement in the tensile properties of magnesium alloys, it is necessary to have at least 0.4 per cent zirconium present in the truly alloyed or available form. However, G. A. Mellor (Journal of the Institute of Metals, 1950, 77, 163) has recently shown that the solubility of zirconium in pure magnesium is only about 0.67%, even at 900° C. I have found that the presence of zinc tends to increase slightly the solubility of zirconium in the alloy, whereas the presence of rare-earth metals tends to decrease the figure quoted by Mellor.

By way of example, an alloying salt within the scope of the present invention made up to contain:

|                   | Per cent |
|-------------------|----------|
| ZrCl <sub>4</sub> | 47       |
| KF                | 23       |
| ZrO <sub>2</sub>  | 20       |
| BaCl <sub>2</sub> | 10       |

was used, according to the technique described hereinbefore, to introduce zirconium into a magnesium alloy containing 4.5 per cent zinc and the resulting alloy was shown, by chemical analysis, to contain 0.7 per cent of soluble zirconium. Similarly, when the same alloying salt was used with a magnesium alloy containing 4.25 per cent mischmetall, the results of the chemical analysis of the cast product showed a soluble zirconium content of 0.57 per cent. Both of the alloys possessed excellent tensile properties and were completely free from salt, flux or dross inclusions.

I wish it to be understood that various changes might be made within the scope of the appended claims, both in respect of the substances used and the steps taken to operate the invention in accordance with this specification.

I claim:

1. Process for alloying of zirconium with magnesium, comprising intimately mixing in the bottom of a warm crucible approximately one part by weight of previously dried potassium fluoride and two parts by weight of zirconium tetrachloride in an amount calculated on the basis of using between 5 and 25% of the total zirconium tetrachloride in the final salt for this purpose, then adding to said bottom layer successive thin alternate layers of zirconium tetrachloride and potassium fluoride, while leaving for the top layer a small amount of the potassium fluoride content, closing said crucible except for a vent hole, gently heating until exothermic reaction occurs, with the production of a molten mass, then stirring into the molten mass the top layer of potassium fluoride thereby forming an alloying salt mixture, said salt mixture comprising a fused mixture of zirconium tetrachloride and potassium fluoride, in which the content of zirconium tetrachloride ranges between 0.75 and 4 parts, by weight, per one part of potassium fluoride, and intimately mixing said salt mixture with molten magnesium.
2. The process of claim 1 wherein the alloying salt contains as an inspissating agent up to 25% of zirconium oxide and wherein at least part of the zirconium oxide is initially mixed with the potassium fluoride and the remainder of the zirconium oxide is mixed as a final step into the molten mass.

References Cited in the file of this patent

| UNITED STATES PATENTS |           |               |               |
|-----------------------|-----------|---------------|---------------|
| 30                    | Number    | Name          | Date          |
|                       | 2,497,538 | Emley et al.  | Feb. 14, 1950 |
|                       | 2,497,551 | Jessup et al. | Feb. 14, 1950 |
| FOREIGN PATENTS       |           |               |               |
| 35                    | Number    | Country       | Date          |
|                       | 533,264   | Great Britain | Feb. 10, 1941 |
|                       | 591,225   | Great Britain | Aug. 12, 1947 |
| 40                    | 624,304   | Great Britain | June 2, 1949  |